

## UNITED STATES PATENT OFFICE

HEINRICH WERDENBERG, OF NEU-ALLSCHWIL, NEAR BASEL, SWITZERLAND, ASSIGNOR  
TO FIRM DURAND & HUGUENIN S. A., OF BASEL, SWITZERLAND

## PROCESS FOR THE PRODUCTION OF COLORED DISCHARGE EFFECTS

No Drawing. Application filed December 16, 1930, Serial No. 502,864, and in Germany December 27, 1929.

Many dyestuffs which are used in hydro-sulphite discharge printing for colored effects show the drawback that after steaming their original dye tone only comes back 5 slowly and not sufficiently deep.

This may be due to the fact that the dye-stuff, which is reduced by the hydrosulphite during the steaming, is only incompletely re-formed on the fibre, perhaps owing to its not 10 being absolutely fast to hydrosulphite and its being partially destroyed.

With a view to completely develop a dye-stuff which is not completely developed, i. e. to 15 oxidize any available leuco compound on the fibre, it is often suggested to submit the material, after the steaming, to an after-treatment in an oxidizing bath containing bichromate of soda or hydrogen peroxide, etc.

Such an aftertreatment is not sufficient in 20 every case and is not applicable to all fibres. Many tones suffer for instance from a treatment with bichromate. Such a treatment is 25 also complicated and costly.

It has now been found that deep effects can be obtained in the direct way by adding to 25 the discharge color a suitable oxidizing agent, such as for instance chlorate (chlorate of soda, chlorate of potash etc.).

It is surprising that a reducing agent like 30 hydrosulphite and an oxidizing agent like chlorate, which are both contained in the printing color at the same time, have no disturbing effect on each other.

The presence of chlorate in the printing 35 paste does not adversely affect the stability of the same. The discharge effect of the ground color is normal and the colored discharges obtained are deeper than those obtained without chlorate.

The present process is applicable to the 40 most different textile fibers. It is explained by the following examples:

## (A) Cotton

The following printing colors are prepared:

|                                              | Parts |
|----------------------------------------------|-------|
| (1) Chromorhodine BR (Colour Index No. 762)  | 20    |
| Hot water                                    | 180   |
| Gum dragon thickening                        | 600   |
| Heat up to dissolve, let cool down and add:  | 55    |
| Sodium - sulphoxylate - formaldehyde         | 100   |
| Chromium acetate 32° Tw                      | 60    |
| Sodium chlorate solution 1:3                 | 40    |
|                                              | 1000  |
| (2) Thiopyronine (Colour Index No. 739)      | 20    |
| Monoethylglycol                              | 50    |
| Hot water                                    | 170   |
| Arabic gum 1:1                               | 500   |
| Heat up to dissolve, let cool down and add:  | 70    |
| Sodium - sulphoxylate - formaldehyde         | 100   |
| Tannin and water 1:1                         | 120   |
| Sodium chlorate solution 1:3                 | 40    |
|                                              | 75    |
| (3) Rhodamine B extra (Colour Index No. 749) | 20    |
| Monoethylglycol                              | 50    |
| Hot water                                    | 170   |
| Arabic gum 1:1                               | 500   |
| Heat up to dissolve, let cool down and add:  | 85    |
| Sodium - sulphoxylate - formaldehyde         | 100   |
| Tannin and water 1:1                         | 120   |
| Sodium chlorate solution 1:3                 | 40    |
|                                              | 90    |

Cotton which is dyed with a dischargeable dyestuff, is printed with one of these discharge colors, dried, aged for 5 minutes in the rapid ager, and afterwards steamed for 40 minutes. In the case of Example 1, there is washed straight away, whereas in the case of Examples 2 and 3 a treatment in a tartar emetic bath takes place before washing. In all three

cases brighter and deeper discharge effects are obtained than with discharge colors which do not contain any chlorate of soda.

(B) Wool

5 The following printing pastes are prepared:

10 (4) Rhodamine B extra (Colour Index No. 749)-----

Monoethylglycol-----  
Hot water-----  
British gum 1:1-----

15 Heat up to dissolve, let cool down and add:

Sodium - sulphonylate - formaldehyde-----  
Sodium chlorate solution 1:3-----

20 -----  
1000 Parts

25 (5) Fast acid violet A2R (Colour Index No. 758)-----

Hot water-----  
British gum 1:1-----

30 Heat up to dissolve, let cool down and add:

Sodium - sulphonylate - formaldehyde-----  
Sodium chlorate solution 1:3-----

35 -----  
1000 Parts

40 (6) Eosine (blue shade) No. 55 (Colour Index No. 778)-----

Hot water-----  
British gum 1:1-----

45 Heat up to dissolve, let cool down and add:

Sodium - sulphonylate - formaldehyde-----  
Sodium chlorate solution 1:3-----

50 -----  
1000 Parts

55 Wool which has previously been dyed with a dischargeable dyestuff is printed with one of these discharge colors, dried, aged in the damp state for 5 minutes in the rapid ager, and steamed afterwards for 40 minutes, then washed. One obtains colored discharge effects which are considerably deeper than those obtained with a printing color which does not contain any chlorate.

(C) Silk

60 The following printing colors are made up:

65 (7) Thiopyronine (Colour Index No. 739)-----

Monoethylglycol-----  
Hot water-----  
Arabic gum 1:1-----

Heat up to dissolve, let cool down and add:

Sodium - sulphonylate - formaldehyde containing zinc oxide-----  
Sodium chlorate solution 1:3-----

150  
40 70

1000

Parts

8 (8) Rhodamine B extra (Colour Index No. 749)-----

Monoethylglycol-----  
Hot water-----  
Arabic gum 1:1-----

75  
50  
140  
600

Heat up to dissolve, let cool down and add:

Sodium - sulphonylate - formaldehyde containing zinc oxide-----  
Sodium chlorate solution 1:3-----

150  
40

1000

Parts

(9) Acridine red brown (German Patent No. 495,115)-----

Monoethylglycol-----  
Hot water-----  
Arabic gum 1:1-----

20  
50  
140  
600

Heat up to dissolve, let cool down and add:

Sodium - sulphonylate - formaldehyde containing zinc oxide-----  
Sodium chlorate solution 1:3-----

150  
40

1000

Parts

(10) Thionine blue GO (Colour Index No. 926)-----

Hot water-----  
Arabic gum 1:1-----

20  
190  
600

Heat up to dissolve, let cool down and add:

Sodium - sulphonylate - formaldehyde containing zinc oxide-----  
Sodium chlorate solution 1:3-----

150  
40

1000

Parts

(11) Eosine (blue shade) No. 55 (Colour Index No. 778)-----

Hot water-----  
Arabic gum 1:1-----

20  
190  
600 115

Heat up to dissolve, let cool down and add:

Sodium - sulphonylate - formaldehyde containing zinc oxide-----  
Sodium chlorate solution 1:3-----

150  
40 120

1000

Silk which has previously been dyed with a dischargeable dyestuff is printed with one of these discharge colors, dried, aged for 5 minutes in the rapid ager, afterwards steamed for 40 minutes and washed. One obtains brighter and deeper discharge effects than when using discharge colors which do not contain any chlorate of soda.

120

(D) *Acetate silk*

The following printing paste is prepared:  
Parts

|                                        |      |
|----------------------------------------|------|
| (12) Thiopyronine (Colour Index No.    |      |
| 5 739)                                 | 30   |
| Monoethylglycol                        | 50   |
| Hot water                              | 90   |
| Arabic gum 1:1                         | 600  |
| Heat up to dissolve, let cool down and |      |
| 10 add:                                |      |
| Sodium - sulphoxylate - formalde-      |      |
| hyde containing basic zinc oxide..     | 150  |
| Sodium chlorate solution 1:3-----      | 80   |
|                                        | 1000 |

15 Acetate silk which has previously been dyed with a dischargeable dyestuff, is printed with the above discharge color, dried, aged for 5 minutes in the rapid ager, and steamed afterwards for 40 minutes, then washed. One obtains a considerably deeper shade than when using a discharge color which does not contain any chlorate of soda.

20 What I claim is:—

25 1. A process for obtaining color discharge effects according to the principle of reduction, consisting in adding to the usual discharge printing color with the view of obtaining color discharge effects of increased 30 intensity together with the reducing agent a chlorate as oxidizing agent.

2. A process for obtaining color discharge effects according to the principle of reduction, consisting in adding to the usual discharge printing color with the view of obtaining colored discharge effects of increased 35 intensity together with the reducing agent sodium chlorate as oxidizing agent.

In witness whereof I have hereunto signed  
40 my name this 6th day of December, 1930.

HEINRICH WERDENBERG.

45

50

55

60

65